

# UNITED STATES PATENT OFFICE.

ROWLAND BRITTAINE MITCHELL, OF ATHOL, MASSACHUSETTS, ASSIGNOR TO ATHOL MANUFACTURING COMPANY, OF ATHOL, MASSACHUSETTS, A CORPORATION OF MASSACHUSETTS.

## SOLVENT FOR PYROXYLIN BODIES.

1,398,239.

Specification of Letters Patent. Patented Nov. 29, 1921.

No Drawing.

Application filed September 22, 1920. Serial No. 411,960.

To all whom it may concern:

Be it known that I, ROWLAND BRITTAINE MITCHELL, a citizen of the United States, residing at Athol, county of Worcester, and 5 State of Massachusetts, have invented a new and useful Improvement in Solvents for Pyroxylin Bodies, of which the following is a full, clear, and exact description.

The object of my invention is to provide 10 a solvent for pyroxylin bodies that will be powerful, complete, and commercially practical and possess the capacity of depositing an odorless, tough, homogeneous and non-hygroscopic film of pyroxylin free from 15 bubbles.

A further object is to provide a pyroxylin solvent in which one of the active ingredients is a solid which will remain in the deposited film after the other liquid ingredients have evaporated, thereby imparting greater toughness and also a certain pliability to the film.

A further object is to provide a pyroxylin solvent of such a nature that certain softening agents, such as castor or rapeseed oil, and certain coloring matters, such as drop black and zinc oxid, can be added to the pyroxylin solution without in any way destroying its usefulness.

30 Naturally, a solvent possessing the above qualities would fill a demand in the pyroxylin industries, such as in the manufacture of artificial leather, lacquers, varnishes and the like. None of the solvents now in 35 use at the present time possesses all of the above qualities. For instance, a well known commercial solvent mixture consisting of ethyl acetate and benzol, toluol or benzin, is apt in humid weather to deposit a hygroscopic film of nitrocellulose. This hygroscopic quality is very objectionable and is evidenced by a whitish appearance in the film, which is caused by the nitrocellulose being precipitated from solution by the wa-

40 ter which is deposited on the surface of the film due to the rapid cooling effect of the evaporation of the solvents. The film's deposited by various well known solvent mixtures are also apt to contain bubbles or pin 45 holes, which are particularly obstructive to the production of a satisfactory piece of artificial leather. For economy it is customary to add cheap diluents to solvents so as to attenuate their solvent power over the 50 greatest possible amount of nitrocellulose.

For instance, in some lacquer work, a solution containing as little as four ounces of pyroxylin to the gallon of solvent will produce a satisfactory film, whereas in some artificial leather work as high as twenty 60 four ounces per gallon are used. Naturally that solvent which will stand the greatest amount of dilution is the preferable one from a commercial standpoint, as the diluents are generally much cheaper than the 65 solvents. However, as a general rule, the more diluent added, the less the solvent power of the resultant solution and the more liability to blushing of the deposited film. Amyl acetate possesses desirable qualities as 70 a solvent, but on account of its high cost is commercially impractical.

In the past it has been customary to use liquid solvents only, where a solution of more or less fluidity has been desired.

75 I have discovered that it is possible to impart great solvent power to a mixture of alcohol (either methyl, ethyl, or butyl) and benzol (or toluol or xylol) by the addition of a relatively small quantity of acetanilid 80 and some other solvent such as acetone, ethyl acetate, methyl acetate, or ethyl propionate. A solvent mixture composed of the above mentioned ingredients not only possesses remarkable solvent power and cheapness, but 85 a pyroxylin solution obtained by using this solvent mixture deposits a film which is non-hygroscopic, odorless, and free from bubbles or pinholes. Acetanilid, having a boiling point of 305°, is left in the deposited 90 film, and its presence there after the other components have evaporated tends to prevent the precipitation of the nitrocellulose through the absorption of the water from the atmosphere. This also tends to produce a 95 tougher and more homogeneous film. This fact also enables the solution to stand a larger quantity of water without precipitating the cellulose.

100 My solvent mixture is commercially practicable because of the ease of manipulation and cheapness due to the large percentage of benzol or equivalent diluent which can be used with it.

The pyroxylin solution made from my 105 solvent mixture possesses a texture which enables it to be painted or spread very smoothly without the bubbles or pinholes usually encountered. This is brought about by the degree to which the solution is carried 110

by this solvent, causing the mixture to become very cohesive and enabling it to be spread or painted evenly.

The following is an example of a solvent mixture embodying my invention:

|            |    |                  |
|------------|----|------------------|
| Benzol     | 72 | parts by weight. |
| Alcohol    | 20 | " "              |
| Acetone    | 6  | " "              |
| Acetanilid | 2  | " "              |

10 The above is typical formula only, the invention not being confined to the specific ingredients or the particular proportions specified.

15 Increasing the amount of acetanilid will result in increased solvent power.

While I mention acetone specifically, I find that other solvents, such as amyl acetate, ethyl acetate, methyl acetone, methyl acetate, 20 acetone oil, ethyl propionate, ethyl butyrate and methyl butyrate, may be used equally well with the other three ingredients without materially changing the properties of the resultant solvent mixtures.

25 In place of benzol any of the other low boiling homologues of the benzene series may be used, as toluol or xylol.

Many other of the aliphatic alcohols may be used instead of ethyl alcohol and the term 30 alcohol therefore includes methyl, ethyl, butyl, propyl, amyl, etc.

While I prefer to use the four ingredients specified in the illustrative composition or their described equivalents, my invention. 35 does not require their employment in the proportions recited; nor does it exclude the addition of other ingredients; nor is it essential to use all the ingredients (or their equivalents) specified to secure results approximating those obtained by the use of 40 the preferred composition. For example, any diluent or diluents, or any ingredient or ingredients functioning mainly as a diluent, may be employed with a plurality of solvents, one of which is acetanilid and the other 45 of which is a solvent boiling at a relatively low temperature. For acetanilid may be substituted any ingredients that is a good solvent

50 vent of pyroxylin, that has a high boiling point, that will remain on the deposited film after the other ingredients have evaporated and that will effect the deposition of an odorless, non-hygroscopic film.

Having now fully described my invention, what I claim and desire to protect by Letters 55 Patent is—

1. A pyroxylin solvent mixture containing a preponderating proportion of an ingredient functioning mainly as a diluent, and a plurality of ingredients, functioning chiefly as 60 solvents, one of which is acetanilid.

2. A pyroxylin solvent mixture containing a preponderating proportion of an ingredient functioning mainly as a diluent, and relatively small proportions of two pyroxylin solvents, one of which has a relatively low boiling point and the other of which has a relatively high boiling point and will remain in the deposited film after the other ingredients have evaporated. 70

3. A pyroxylin solvent mixture containing a preponderating proportion of an ingredient functioning mainly as a diluent, a relatively small proportion of an aliphatic alcohol, and a still smaller proportion of a plurality of solvents one of which is acetanilid. 75

4. A pyroxylin solvent mixture containing a material which is a good solvent of pyroxylin, alcohol, a lower member of the benzene series of hydrocarbons, and acetanilid. 80

5. A pyroxylin solvent mixture containing alcohol, a material which is a solvent of pyroxylin in a proportion substantially less than the proportion of alcohol, acetanilid in a proportion substantially less than the proportion of alcohol, and a diluent in a proportion substantially in excess of all the other ingredients combined. 85

6. A pyroxylin solvent mixture containing acetone, an aliphatic alcohol, a lower member of the benzene series of hydrocarbons and acetanilid. 90

In testimony of which invention, I have hereunto set my hand, at Athol, Mass., on this 16 day of August, 1920.

ROWLAND BRITAIN MITCHELL.